

## UNITED STATES PATENT OFFICE

2,258,930

## METAL DRAWING PROCESS

Rudolf Haefner, Frankfort-on-the-Main-Romerstadt, and Max Schunck, Oberursel, near Frankfort-on-the-Main, Germany

No Drawing. Application January 21, 1939, Serial No. 252,208. In Germany January 25, 1938

2 Claims. (Cl. 205—21)

In the cold drawing of tubes or pipes, rods, bars and profiles from metals which are difficult to draw and which deposit easily in the drawing iron or draw plate, for example, iron, nickel and their alloys or platings of these metals and other metals, for example, copper, it has already been proposed in order to facilitate the work of drawing to put upon the tubes or body to be drawn before the drawing, a surface protecting layer, which prevents the direct contact of the tube or body and die, thereby preventing the deposition of metal in the hollow of the draw plate. Ordinarily these protecting layers are of a metallic nature, and are produced by metallizing the pieces of metal to be worked by immersion in molten baths, or by immersion in metal salt solutions preferably accompanied by electrolysis, or by boiling processes. In these ways, layers or coatings of lead, tin and copper, for example, have been applied to the pieces of metal. Coatings of a non-metallic kind, which are applied in the form of a paint upon the pieces to be worked, are seldom used. With all of these coatings it is necessary in conjunction with the drawing process to use a drawing fat or drawing oil, in order to reduce the friction in the dies.

The present invention relates to a non-metallic coating medium, and to process for drawing metal, which prevents deposit in the dies, which simultaneously effects lubrication, which does not require the addition or use of drawing fat and the like, which is extremely simple to use or operate and which, at the same time, is comparatively inexpensive. A particular and surprising advantage of the present invention resides in that the coatings according to the present invention, after having been preliminarily applied to the metal to be drawn, are able thereafter to bear or experience several successive drawing operations of the metal without it becoming again necessary, between the separate or individual drawings, to treat the surface of the metal to be drawn. For example, iron tubing of 2.5 mm. wall thickness, after having been coated according to the present invention, is able to be drawn or stretched in three successive drawing operations, without intermediate annealing, to a wall thickness of 1.0 mm. and without it being or becoming necessary to repeat the treatment of the metal with the drawing composition according to the invention.

The invention utilizes pure bitumen, for example petroleum bitumen. Such form of bitumen, of course, has not been heated with sulphur to sulphurize it. The softening point of the bitumen to be used according to the present invention can be chosen between 20 and 100° Celsius according to the metal to be drawn and the degree of cross section reduction or the number of drawing operations or pulls which are to be

undertaken in succession. For example, in drawing hard steel, or when many successive draws without intermediate treatment are to be performed, bitumens with a softening point between 60 and 100° Celsius are chosen, while in drawing softer metals, such as iron, bitumens with a softening point below 60° Celsius are employed advantageously.

The manner of applying the bitumen to the surfaces of the metal pieces to be drawn is as follows: the solid bitumen is dissolved in a suitable solvent, for example, benzine, and the pieces of metal are then treated with the solution by dipping them in the solution or coating the solution upon them. After evaporation of the solvent, the actual drawing of metal pieces can then be performed in a suitable known manner.

Especially good results are also obtained when bitumens of high softening point are employed if their softening points have been lowered by the addition of mineral, vegetable or animal oils and fats, for example, paraffin oil. The following are given as examples of coating compositions suitable for use according to the present invention:

|                                                 | Kilograms |
|-------------------------------------------------|-----------|
| (1) Petroleum bitumen of 55° C. softening point | 50        |
| Benzine                                         | 50        |
| (2) Petroleum bitumen of 70° C. softening point | 50        |
| Paraffin oil                                    | 5         |
| Benzine                                         | 45        |

## 35 We claim:

1. The process which comprises applying to metal to be drawn a coating composition comprising a solution of a non-sulphurized bitumen of 20° to 100° Celsius softening point in about an equal weight of a volatile solvent for the bitumen, and after evaporation of volatile solvent from the said applied composition, subjecting the so treated metal to a drawing operation.

2. The process which comprises applying to metal to be drawn a coating composition comprising a solution, in a volatile solvent of a solid non-sulphurized bitumen and a material which lowers the softening point of the bitumen, a hundred parts by weight of said solution containing about fifty parts by weight of the bitumen, a few parts by weight of the material which lowers the softening point of the bitumen and a few parts less than fifty parts by weight of the volatile solvent; and after evaporation of the volatile solvent from the applied composition, subjecting the so treated metal to a drawing operation.

RUDOLF HAEFNER.  
MAX SCHUNCK.